

1

3,787,458

**OIL-SOLUBLE ALIPHATIC ACID MODIFIED HIGH MOLECULAR WEIGHT MANNICH CONDENSATION PRODUCTS**

Edmund J. Piasek, Chicago, and Robert E. Karl, Batavia, Ill., assignors to Standard Oil Company, Chicago, Ill.  
No Drawing. Continuation-in-part of application Ser. No. 54,558, July 13, 1970. This application Aug. 31, 1970, Ser. No. 68,469

Int. Cl. C09f 7/00

U.S. Cl. 260—404.5

10 Claims

**ABSTRACT OF THE DISCLOSURE**

The thermal oxidation stability of aliphatic acid-modified high molecular weight Mannich condensation products, which are prepared by reacting (1) a high molecular weight alkyl-substituted hydroxy aromatic compound, in which the alkyl-substituent has an average molecular weight of from about 600 to about 100,000, (2) an amine compound containing at least one  $\text{HN}^+$  group, (3) an aliphatic aldehyde, and (4) an aliphatic acid containing at least six carbon atoms, in the reactant molar ratio of 1:0.1-10:1-10:0.014-1.0, respectively, are improved by reacting such modified Mannich condensation products with from about 2 to about 6 moles of an aliphatic aldehyde per mole of the alkyl-substituted hydroxy aromatic compound used in preparing the modified Mannich condensation product. The products of the herein-described invention are oil-soluble, and are highly effective additives for imparting dispersant-detergent properties to lubricant oil compositions. Lubricants containing these products provide a high degree of protection against the deposition of sludge and varnish, and corrosion when used as crankcase lubricant additives.

**RELATED APPLICATIONS**

This application is a continuation-in-part of our co-pending application Ser. No. 54,558, filed July 13, 1970.

**BACKGROUND OF THE INVENTION**

This invention relates to improved lubricating oils and particularly concerns automobile and diesel crankcase lubricating oil formulations containing a minor amount of a new class of oil-soluble addition agents which improve the performance of the oil, particularly its dispersant-detergent function thus enabling lubricating oils to provide a high degree of protection of the lubricated parts of internal combustion engines.

Present-day automobile and diesel engines have been designed for higher power output, lower combustion products emission and longer in-service periods of use of crankcase lubricating oils. These design changes have resulted in such severe operating conditions as to necessitate devising higher efficiency lubricating oils that will, under the increased severity of in-service use, afford proper protection against corrosion and the accumulation or deposition of sludge, varnish and resinous materials on the surface of engine parts which rapidly accelerate decrease in both operating efficiency and life of the engine. The principal ingredient of crankcase lubricants is a base lubricating oil, a mixture of hydrocarbons derived from petroleum. Even when highly refined by removal of deleterious components, such as polymerizable components, acid formers, waxes, etc., a lubricant base oil still requires the addition of a number of oil-soluble chemical additives to enable the oil to resist oxidation, deposition of sludge and varnish on, and corrosion of, the lubricated metal parts, and to provide added lubricity and regulated viscosity change from low to high temperature.

2

These ingredients are commonly known as anti-oxidants, dispersant-detergents, pour point dispersants, etc.

Combustion products from the burning of fuel and thermal degradation of lubricating oils and addition agents tend to concentrate in the crankcase oil with the attendant formation of oil-insoluble deposit-forming products, that either surface coat the engine parts (varnish or lacquer-like films) or settle out on the engine parts as viscous (sludge) deposits or form solid ash-like or carbonaceous deposits. Any of such deposits can restrict, and even plug, grooves, channels and holes provided for lubricant flow to the moving surfaces of the engine requiring lubrication thus accelerating the wear and thus reducing the efficiency of the engine. In addition, acidic combustion products corrode the lubricated metal surfaces. Chemical additives are blended in crankcase oil formulations not only to reduce thermal decomposition of the oil and addition agents (antioxidants) but also to keep in suspension (as a dispersant) and to resuspend (as a detergent) insoluble combustion and degradation products as well as to neutralize acidic products (anti-corrosion agents). A separate additive is usually added for each improvement to be effected.

As performance levels increased and recommended periods between oil drains lengthened for both automobile and railway diesel engines, more efficient dispersancy and detergency performance, as well as better acid neutralization and lower ash-forming properties were demanded for lubricating oil formulations. Among additives suggested by the prior art are amine salts, amides, imides, and amidines of polybutenyl-substituted polycarboxylic acids and polymeric compounds having pendant or grafted-on polar groups. Other suggested prior additives are combinations of alkaline earth metal sulfonates and Mannich condensation products of low molecular weight alkyl ( $C_2-C_{20}$ ) substituted hydroxyaromatic compounds, amine having at least one replaceable hydrogen on a nitrogen and aldehydes; and alkaline earth metal salts of such Mannich condensation products. These prior art products did not provide the desired dispersancy-detergency properties and possessed the objectionable property of forming harmful metal-ash deposits.

Mannich condensation products derived from alkyl-substituted hydroxyaromatic compounds having a relatively low molecular weight alkyl substituent, i.e., 2 to 20 carbon atoms in the alkyl substituent and chlorinated wax (straight chain) type alkyl-substituents are described in U.S. Pat. Nos. 2,403,453; 2,353,491; 2,363,134; 2,459,112; 2,984,550 and 3,036,003. However, none of such prior Mannich condensation products are suitable for use as dispersant-detergent addition agents for present-day long drain oil interval in-service use.

One known type (U.S. Pat. No. 2,363,134) has been prepared by reacting, under Mannich reaction conditions, equimolar quantities of a  $C_2-C_{20}$  alkyl-substituted phenol and other hydroxy aromatic compounds, and  $N,N$ -di-substituted amine and formaldehyde.

The prior  $C_2-C_{20}$  alkyl-substituted Mannich condensation products commonly are prepared by the conventional technique of adding the aliphatic aldehyde to a heated mixture of the alkylhydroxyaromatic and amine reagents, in the presence or absence of a solvent, and then heating the resultant mixture to a temperature between 100-350° F. until dehydration is complete. A solvent such as benzene, toluene, xylene, methanol and others easily separated from the reaction mixture and light mineral oils, such as those used in blending stocks to prepare lubricating oil formulations in which the product is formed as a mineral oil concentrate are usually used. The water by-product is removed by heating the reaction mixture to a temperature sufficiently high, at

least during the last part of the process, to drive off the water alone, or as an azeotropic mixture with the aromatic solvent, usually by the aid of an inert stripping gas, such as nitrogen, carbon dioxide, etc.

The neutralized or overbased alkaline earth metal salts (alkaline earth metal phenates) of those prior low molecular weight Mannich condensation products have been suggested for use in providing lubricating oils with a combination of detergent-inhibitor properties in one addition agent. The neutralized alkaline earth metal salts have one equivalent of alkaline earth metal for each hydroxy group present. The overbased salts have, for each hydroxy group present, more than one equivalent of alkaline earth metal in the form of a hydroxy metaloxy, alkoxy metaloxy and even alkaline earth metal carbonate complex with hydroxy metaloxy on each benzene group as a replacement for the phenol hydroxy group. As noted above, said addition agents form objectionable metal ash deposits and have other performance deficiencies.

U.S. Pat. No. 3,368,972, issued Feb. 13, 1968, describes as dispersant-detergent addition agents for lubricating oils high molecular weight Mannich condensation products from (1) high molecular weight alkyl-substituted hydroxyaromatic compounds whose alkyl-substituent has a molecular weight in the range of 600-3000, (2) a compound containing at least one  $\text{HN}^<$  group and (3) an aldehyde in the respective molar ratio of 1.0:0.1-10:1.0-10.

The high molecular weight Mannich condensation products of U.S. Pat. No. 3,368,972 have a drawback in their large-scale preparation and in their extended service use as lubricant addition agents used under high temperature conditions such as encountered in diesel engines. In the large-scale or plant preparation of such high molecular weight condensation products, especially in light mineral oil solvents, the resulting oil concentrate solution of the condensation product either has or develops during storage a haze which is believed to be caused by undissolved or border line soluble by-products which not only are substantially incapable of removal by filtration but also severely restrict product filtration rate. When used in diesel engine crankcase lubricant oils and subject to high temperature in service use, piston ring groove carbonaceous deposits and skirt varnish tend to build up sufficiently rapidly and prevent desirable long in-service use of such lubricant oils.

As taught and claimed in our aforesaid co-pending application, both of these drawbacks are overcome by modifying the high molecular weight Mannich condensation products with an aliphatic acid having at least six carbon atoms. While such modification of such Mannich condensation products overcomes the aforementioned drawbacks, such modified Mannich products do not possess the desired thermal oxidation stability. We have now discovered that the storage and thermal stability of such aliphatic acid-modified high molecular weight Mannich condensation products are improved by treating such condensation products with an additional amount of an aliphatic aldehyde.

#### BRIEF SUMMARY OF THE INVENTION

This invention pertains to a new class of compounds useful as multifunctional addition agents for lubricating oils, particularly such oils used in internal combustion engines in which they function as highly efficient dispersant-detergent and oxidation inhibitor agents.

The new class of compounds which comprise our invention are oil-soluble high molecular weight Mannich condensation products, which are further treated with an aliphatic aldehyde. They can be made by condensing in the usual manner under Mannich reaction conditions at a temperature in the range of 150-325° F.

(1) An alkyl-substituted hydroxyaromatic compound, in which the alkyl-substituent has an average molecular weight of about 600-100,000, preferably a polyalkylphenol whose polyalkyl substituent is derived from 1-monoolefin polymers having an average molecular weight of about 850-2500;

(2) An amine containing at least one  $>\text{NH}$  group, preferably an alkylene polyamine of the formula



wherein A is a divalent alkylene radical having 2 to 6 carbon atoms, and x is an integer from 1 to 10;

(3) An aliphatic aldehyde, preferably formaldehyde or paraformaldehyde; followed by reaction with;

(4) A high molecular weight aliphatic acid before or after filtration; or they can be prepared by using all four reactants at one time under the general Mannich reaction conditions.

The above resultant modified Mannich condensation product is then treated with (5) an aliphatic aldehyde in an amount of from about 2 to about 6 moles of the aldehyde per mole of the alkyl-substituted hydroxy compound used in the preparation of said modified Mannich product.

The foregoing high molecular weight products of this invention are preferably prepared according to the conventional methods employed for the preparation of Mannich condensation products, using the first four above mentioned reactants in the respective molar ratios of about 1.0:0.1-10:1.0-10:0.014-1.0. Suitable condensation procedure involves adding at a temperature of from room temperature to about 200° F. the aldehyde reagent (3) to a mixture of reagents (1), (2), and (4), above, or such reagents in an easily removed organic solvent, such as benzene, xylene, or toluene, or in a solvent refined mineral oil; completing the reaction at 300° F.; then slowly adding the additional aldehyde, reactant (5) at 180-300° F. The reaction mass is then heated at an elevated temperature of about 275-375° F., preferably with blowing with an inert stripping gas, such as nitrogen, carbon dioxide, etc. until dehydration is complete.

The preferred additives, according to this invention, are high molecular weight bis-Mannich condensation products formed by reacting (1) a 850-2500 molecular weight polybutylphenol; (2) an ethylene polyamine; (3) formaldehyde; and (4) an aliphatic acid in the respective molar ratio of 1.0:0.7-1.0:1.5-2.1:0.014-0.62, and treating the resultant modified Mannich condensation product with 2-4 moles of paraformaldehyde per mole of the polybutylphenol. The preferred aliphatic acid reactant is an acid having 10-20 carbon atoms per carboxylic acid group.

To those skilled in the art, it will be recognized that, in general, the reaction under Mannich condensation conditions, as in other chemical reactions, does not go to theoretical completion, and some portion of the reactants remain unreacted or only partially reacted as co-products. Accordingly, the products of this invention cannot be properly or accurately characterized with precision by chemical structural formula, but must be characterized as reaction products produced by the method of preparation.

The high molecular weight products of this invention are effective additives for lubricating oil lubricants, imparting thereto dispersant-detergent properties and high temperature oxidation stability, at relatively low concentrations, e.g., 0.05% to about 10% in formulated crankcase lubricating oil compositions. Higher concentrations, e.g., 10% to about 70%, are useful concentrates for the preparation of such lubricating oil compositions.

#### EMBODIMENT OF THE INVENTION

Representative high molecular weight aliphatic acid modified Mannich condensation products contemplated by this invention can be prepared from the following representative reactants of the classes before defined.

## (1) High molecular weight alkyl-substituted Hydroxyaromatics

Representative of these high molecular weight alkyl-substituted hydroxyaromatic compounds are polypropylphenol, polybutylphenol and other polyalkylphenols. These polyalkylphenols may be obtained by the alkylation, in the presence of an alkylating catalyst, such as  $\text{BF}_3$ , of phenol with high molecular weight polypropylene, polybutylene and other polyalkylene compounds to give alkyl substituents on the benzene ring of phenol having an average 600-100,000  $\overline{M}_n$ . Their preparation using a  $\text{BF}_3$  phenol catalyst is described and claimed in our co-pending application Ser. No. 484,758, filed Sept. 2, 1965, now abandoned.

The 600  $\overline{M}_n$  and higher  $\overline{M}_n$  alkyl-substituents on the hydroxyaromatic compounds may be derived from high molecular weight polypropylenes, polybutenes and other polymers of mono-olefins, principally 1-mono-olefins. Also useful are copolymers of mono-olefins with monomers copolymerizable therewith wherein the copolymer molecule contains at least 90%, by weight, of mono-olefin units. Specific examples are copolymers of butenes (butene-1, butene-2 and isobutylene) with monomers copolymerizable therewith wherein the copolymer molecule contains at least 90%, by weight, of propylene and butene units, respectively. Said monomers copolymerizable with propylene or said butenes include monomers containing a small proportion of unreactive polar groups such as chloro, bromo, keto, ether, aldehyde, which do appreciably lower the oil-solubility of the polymer. The co-monomers polymerized with propylene or said butenes may be aliphatic and can also contain non-aliphatic groups, e.g., styrene, methylstyrene, p-dimethylstyrene, divinyl benzene and the like. From the foregoing limitation placed on the monomer copolymerized with propylene or said butenes, it is abundantly clear that said polymers and copolymers of propylene and said butenes are substantially aliphatic hydrocarbon polymers. Thus the resulting alkylated phenols contain substantially alkyl hydrocarbon substituents having  $\overline{M}_n$  upward from 600.

In addition to these high molecular weight hydroxyaromatic compounds others which may be used include those which have been used to prepare prior low molecular weight Mannich condensation products, e.g., high molecular weight alkyl-substituted derivatives of resorcinol, hydroquinone, cresol, catechol, xylenol, hydroxy diphenyl, benzylphenol, phenethylphenol, naphthol, tolylnaphthol, among others. Preferred for the preparation of the aforementioned preferred bis Mannich condensation products are the polyalkylphenol reactants, e.g., polypropylphenol and polybutylphenol whose alkyl group has an average number molecular weight of 600-3000, the most preferred being polybutylphenol whose alkyl group has an average number molecular weight of 850-2500.

(2)  $\text{HN} <$  group containing reactants

Representative of this class of reactants are alkylene polyamines, principally polyethylene polyamines. Other representative organic compounds containing at least one  $\text{HN} <$  group suitable for use in the preparation of Mannich condensation products are well known and include the mono- and di-amino alkanes and their substituted analogs, e.g., ethylamine and diethanol amine; aromatic diamines, e.g., phenylene diamine, diamino naphthalenes; heterocyclic amines, e.g., morpholine, pyrrole, pyrrolidine, imidazole, imidazolidine, and piperidine; melamine and their substituted analogs.

Suitable alkylene polyamine reactants include ethylenediamine, diethylene triamine, triethylene tetramine, tetraethylene pentamine, pentaethylene hexamine, hexaethylene hepta-amine, heptaethylene octamine, octaethylene nonamine, nonaethylene decamine and decaethylene undecamine and mixture of such amines having nitrogen contents corresponding to the alkylene polyamines, in the formula  $\text{H}_2\text{N}-(\text{A}-\text{NH})_x\text{H}$ , mentioned before, A is

divalent ethylene and x is 1 to 10 of the foregoing formula. Corresponding propylene polyamines such as propylene diamine and di-, tri-, tetra-, penta-propylene tri-, tetra-, penta- and hexa- amines are also suitable reactants. The alkylene polyamines are usually obtained by the reaction of ammonia and dihalo alkanes, such as dichloro alkanes. Thus the alkylene polyamines obtained from the reaction of 2 to 11 moles of ammonia with 1 to 10 moles of dichloro alkanes having 2 to 6 carbon atoms and the chlorines on different carbons are suitable alkylene polyamine reactants.

## ALDEHYDE REACTANTS

Representative of this aldehyde class of reactants for use in the preparation of the high molecular products of this invention include the aliphatic aldehydes such as formaldehyde (also as paraformaldehyde and formalin), acetaldehyde and aldol (b-hydroxybutyraldehyde). We prefer to use formaldehyde, para-formaldehyde or a form-aldehyde yielding reactant.

## ALIPHATIC ACID REACTANTS

The aliphatic acid reactant of this invention has a carbon atom content of a total (including the carbon of the carboxylic acid group) of from about six to about 30 and consists of the alkanoic (saturated) and alkenoic (mono-unsaturated) acids. The upper limit of the carbon content is restricted only by the largest carbon atom content of such acids available or capable of feasible preparation. Such aliphatic acids can be natural and synthetic mono-, di- and tri-carboxylic acids. Suitable natural aliphatic acids are the natural fatty acids obtainable by known hydrolysis (acid and alkaline) of vegetable and animal oils and fats and wax esters. Of those natural acids for the purposes of this invention the preferred acids have from 10 to about 20 total carbon atoms per carboxylic acid group. Suitable synthetic acids can be derived from oxidation of the alcohol moiety of the wax ester where such alcohol moiety has at least six carbon atoms; from the polymerization of unsaturated natural acids having two or three carbon to carbon double bonds (dimer and trimer acids) and the hydrogenation of residual carbon to carbon double bonds in such polymer acids. For example the polymer acids obtained from oleic acid, uric acid, linoleic acid and linolenic acid and other unsaturated acids; and from oxidation or other reactions of polypropenes and polybutenes (e.g. polyisobutenes) which introduce one or more carboxylic acid group on the polymer chain.

It might be expected that the high molecular weight Mannich product modified by an unsaturated aliphatic carboxylic acid such as oleic acid or its  $\text{C}_{16}$  unsaturated homolog would have less oxidation stability than for example such Mannich products modified by a saturated aliphatic acid such as stearic acid. But this, somewhat unexpectedly, is not the case. For example, in a standard oxidation stability test (Union Pacific Oxidation Test) there are tested oil formulations containing equivalent amounts of high molecular weight Mannich product (a polybutyl-, hydroxybenzyl-substituted tetraethylene pentamine having a number average molecular weight of 3600) and the same Mannich product modified with 0.125 mole (0.8 weight percent) of each of oleic acid, isostearic acid, a mixture of  $\text{C}_{16}$  and  $\text{C}_{18}$  monounsaturated alkenoic acids and a mixture of  $\text{C}_{16}$  and  $\text{C}_{18}$  saturated alkanoic acids. The pentane insolubles content of these tests, indicative of oxidation stability, is measured and is as follows:

| Additive        | Acid modifier                                                   | Pentane insolubles, gms. |
|-----------------|-----------------------------------------------------------------|--------------------------|
| Mannich product | None                                                            | 1.5                      |
| Do              | Oleic acid                                                      | 2.5                      |
| Do              | Isostearic acid                                                 | 3.0                      |
| Do              | $\text{C}_{16}-\text{C}_{18}$ mixtures of monounsaturated acids | 3.0                      |
| Do              | $\text{C}_{16}-\text{C}_{18}$ mixture of saturated acids        | 2.0                      |

Suitable alkanoic acids having 6 or more total carbon atoms are those obtainable from the glycerides: vegetable oils and animal fats and the wax esters by the known hydrolysis or saponification-acidification or acid treatment processing of said oil and fat glycerides and the wax esters (i.e. natural waxes), the oxidation of the mono-alcohol obtainable from the simple ester of the wax esters and known acid synthesis. Such suitable alkanoic acids, i.e. having R groups of 6 to 30 carbon atoms, include caproic acid, caprylic acid, capric acid, heptadecylic acid, lauric acid, tridecyllic acid, myristic acid, pentadecylic acid, palmitic acid, margaric acid, stearic acid, nonadecylic acid, arachidic acid, medullic acid, behenic acid, lignoceric acid, pentacosic acid, cerotic acid, heptacosic acid, monocosic acid, montanic acid, and melissic acid. Many of said alkanoic acids are obtained first in mixtures of two, three or more alkanoic acids of different carbon contents from said glycerides and wax esters; said mixtures can be used in this invention in place of a single alkanoic acid reactant. When said mixtures of alkanoic acids also contain unsaturated acids it is preferred that such mixture of acids be reduced to a product which is substantially free of unsaturation.

Suitable alkenoic acids having a total of at least six carbon atoms include those from hexenoic, heptenoic, octenoic, etc. acids up to oleic ( $C_{18}$ ) and erucic ( $C_{22}$ ) acids. Also suitable are the dimer acid of linoleic and its saturated dimer analog; dimer and trimer acids of linolenic acid and the saturated dimer and trimer analogs. Other polymeric acids, e.g. co-dimers of oleic and linoleic or linolenic acids and the saturated analogs of those dimer acids are also suitable.

The foregoing, while not an exhaustive listing of all suitable aliphatic acid reactants of the class before defined, will provide adequate guidance for the chemist skilled in this art and also bring to mind other suitable aliphatic acids within the scope before defined.

The following examples are illustrative of preferred embodiments of the present invention.

#### EXAMPLE I

2085 grams (0.61 mole) of a 1600 average molecular weight polybutyl-substituted phenol (47% polybutylphenol, 53% polybutene and diluent oil), 765 grams of a solvent-extracted 5W mineral oil, 109 grams (0.56 mole) tetraethylene pentamine, and 109 grams (0.38 mole) of a modified saturated  $C_{16}$ - $C_{18}$  fatty acid, identified as "Emery 896 Fatty Acid" by Emery Industries Inc., were admixed and heated to 150° F. 84 ccs. (1.12 moles) of formalin were then rapidly added to the mixture. Thereafter, there were slowly added 168 ccs. (2.24 moles) of formalin over a 1.5 hour period, during which time the reaction temperature was allowed to rise to 200-220° F. Upon completion of the formaldehyde addition, the reaction mixture was heated to a temperature of 300-320° F. and held at such temperature for 3 hours while blowing with nitrogen at a rate of 2 cubic feet per hour (c.f.h.). At the end of three hours the reaction mass was filtered. The recovered filtrate was clear, had a nitrogen content of 1.30%, and a SSU viscosity at 210° F. of 954.

#### EXAMPLE II

Part A.—2370 grams (0.73 mole) of a 1526 average molecular weight polybutyl-substituted phenol (49.4% polybutylphenol, 50.6% polybutene and oil), 300 grams of a solvent-extracted 5W mineral oil, 128 grams (0.454 mole) oleic acid, and 127 grams (0.672 mole) tetraethylene pentamine were admixed at 150° F., and 100 ccs. (1.344 moles) formaldehyde added. The temperature was increased to 300-320° F. while blowing with nitrogen at 2 c.f.h., and maintained at such temperature for 2 hours. 489 grams of a solvent-extracted 5W mineral oil were added to the reaction product.

Part B.—To 3200 grams of an oleic acid-modified Mannich condensation product prepared as in part A, above,

were added at 300° F. 90 grams (2.8 moles) paraformaldehyde, and 140 grams of a solvent-extracted 5W mineral oil, and the mixture maintained at 300-320° F. for 3 hours while blowing with nitrogen at the rate of 2 c.f.h. The reaction product was then filtered.

Three other batches were prepared as the above, and the four batches combined. The composite product was crystal clear and had a SSU viscosity at 210° F. of 1028.

The thermal oxidation stability of the aldehyde treated acid-modified high molecular weight Mannich condensation product is demonstrated by the so-called "Hot Tube Test." This test measures the oxidation and thermal stability of dispersant additives for lubricating oils, particularly automotive crankcase lubricants. In making this test the subject dispersant is incorporated in a typical crankcase lubricating oil composition formulation, and the composition subjected to the following test: The oil composition being tested is passed, at the rate of 0.1 cc. per minute downward through a 20 inch, 8 mm. vertical glass tube 6 inches of which are surrounded by a furnace and heated at 495° F. for 100 minutes, while air at the rate of 20 ccs. per minute is passed downwardly through the tube. At the end of the 100 minute test period the tube is cooled and rinsed with hexane, and the appearance of the tube evaluated as to varnish area and intensity. A perfect tube is rated "10A," where the numerical value refers to the varnish in the heated portion of the tube, and the letter rating refers to the varnish formed in the cool zone of the tube below the furnace. The lower the numerical rating and the higher the letter rating, the poorer is the oxidation and thermal stability of the dispersant.

The data in Table I, below, were obtained by subjecting the following lubricating oil formulations to the above "Hot Tube Test":

#### Sample A

|                                                      | Percent (vol.) |
|------------------------------------------------------|----------------|
| Unmodified Mannich condensation product <sup>1</sup> | 4.1            |
| Overbased sulfonate                                  | 2.0            |
| Zinc dialkyl dithiophosphate                         | 1.1            |
| Solvent-extracted 10W mineral oil                    | 70.0           |
| Solvent-extracted 5W mineral oil                     | 22.8           |

<sup>1</sup> This Mannich condensation product was prepared by mixing together 260 grams (0.073 mole) of a 1600 average molecular weight polybutyl-substituted phenol (42% polybutylphenol, 58% polybutene and oil), 39 grams of a solvent-extracted 5W mineral oil, 13 grams (0.067 mole) tetraethylene pentamine, and the mixture heated to 150° F., 10 ccs. (0.134 mole) formalin were then added, and the mixture reacted at 300-320° F. for 3 hours while blowing with nitrogen at the rate of 1 c.f.h. At the end of the reaction period the product was filtered. The filtrate had a SSU viscosity at 210° F. of 1258.

Sample B.—Same as sample A, except that 4.1% of the product of Example II, part A, above, was used. This is an acid-modified Mannich condensation product.

Sample C.—Same as sample A, except that 4.1% of the product of Example II, part B, above, was used. This is the aldehyde treated acid-modified Mannich condensation product of the present invention.

TABLE I

| Sample: | Hot tube rating |
|---------|-----------------|
| A       | 7.8D            |
| B       | 8.2C            |
| C       | 8.0B            |

The letter rating "B" in the above test indicates that the aldehyde treated acid-modified Mannich condensation product (sample C), exhibits better thermal oxidation stability than the acid-modified Mannich product (sample B), which had a letter rating of "C."

As noted hereinbefore, the products of the present invention are useful addition agents for lubricating oils. Such oils can be any normally liquid oleaginous lubricants, such as hydrocarbon oils, both natural, i.e., petroleum oils, and synthetic lubricating oils, for example, those obtained by the polymerization of olefins, as well as synthetic lubricating oils of the alkylene oxide type, and the poly-

carboxylic acid ester type, such as the oil-soluble esters of adipic acid, sebacic acid, azelaic acid, etc.

Lubricating oil compositions containing the aldehyde treated acid-modified Mannich condensation products of the present invention, may also contain other additives such as for example, VI improvers, rust inhibitors, oiliness agents, pour point depressors, etc.

Percentages given herein and in the appended claims are weight percentages unless otherwise stated.

Although the present invention has been described with reference to specific preferred embodiments thereof, the invention is not to be limited thereto, but includes within its scope such modifications and variations as come within the scope and spirit of the appended claims.

We claim:

1. An oil-soluble aliphatic acid-modified high molecular weight Mannich condensation product prepared by the process comprising (A) reacting at a temperature of from about 150° F. to 325° F.:

- (a) a high molecular weight alkyl-substituted phenol wherein the alkyl substituent has an average molecular weight of from about 600 to about 100,000;
- (b) an alkylene polyamine;
- (c) formaldehyde; and
- (d) a higher aliphatic acid containing 10 to 30 carbon atoms, said reactants (a), (b), (c), and (d) being used in the molar ratios of 1.0:0.1-10:1.0-10:0.014-0, respectively, (B) then slowly adding to the resultant foregoing product of (A) at a temperature in the range of 180-300° F.;
- (e) additional formaldehyde in the molar ratio of from about 2 to about 6 moles thereof per mole of said reactant (a), and (C) increasing the temperature of the resultant reaction mass to from about 275° F. to about 375° F. while blowing with an inert stripping gas to dehydrate the resultant product.

2. The oil-soluble aliphatic acid-modified high molecular weight Mannich condensation product of claim 1, wherein the high molecular weight alkyl-substituted hydroxyaromatic compound is a polyalkyl-substituted phenol, wherein the polyalkyl-substituted has a molecular weight of from about 600 to about 3,000.

3. The oil-soluble aliphatic acid-modified high molecular weight Mannich condensation product of claim 2 wherein the alkylene polyamine is tetraethylene pentamine.

4. The oil soluble aliphatic acid-modified high molecular weight Mannich condensation product of claim 2, wherein the additional aldehyde (e) is paraformaldehyde.

5. The oil-soluble aliphatic acid-modified high molecular weight Mannich condensation product of claim 3, wherein the aliphatic acid is oleic acid.

6. An oil-soluble aliphatic acid modified high molecular weight Mannich condensation product prepared by the process comprising, (A) reacting at a temperature of from 150 to 325° F.:

- (a) a high molecular weight alkyl-substituted phenol wherein the alkyl-substituent has an average molecular weight of from about 600 to about 3,000;
- (b) an alkylene polyamine;
- (c) formaldehyde; and
- (d) a higher aliphatic acid containing 10 to 30 carbon atoms, said reactants (a), (b), (c) and (d) being used in molar ratios of 1.0:0.1-10:1.0-10:0.014-1.0, respectively, (B) then slowly adding to the resultant foregoing product of (A) to a temperature in the range of 180-300° F.;
- (e) additional formaldehyde in the molar ratio of from about 2 to about 6 moles thereof per mole of

said reactant (a), and (C) increasing the temperature of the resultant reaction mass to from about 275° F. to about 375° F. while blowing with an inert stripping gas to dehydrate the resultant product.

5 7. The oil-soluble aliphatic acid modified Mannich condensation product of claim 6, wherein the alkyl-substituted phenol (a) is selected from the group consisting of polypropylphenol and a polybutylphenol in which the polypropyl and the polybutyl substituents have average molecular weight of from about 600 to about 3,000, the amine reactant (b) has the formula



15 wherein  $x$  is an integer from 1 to 10, aldehyde (c) is formalin, the aliphatic acid (d) is a fatty acid having from about 10 to about 20 total carbon atoms per carboxylic acid group, and the additional aldehyde (e) is paraformaldehyde.

20 8. The oil-soluble aliphatic acid modified high molecular weight Mannich condensation product of claim 6, wherein the alkyl-substituted phenol is a polybutylphenol (a) in which the polybutyl substituent has an average molecular weight of about 1,500, the alkylene polyamine (b) is tetraethylene pentamine, aldehyde (c) in formalin, the aliphatic acid (d) is oleic acid, and the additional aldehyde (e) is paraformaldehyde.

25 9. A method of preparing the oil-soluble acid-modified high molecular weight Mannich product of claim 1 as solute in the presence of hydrocarbon diluent consisting essentially of aliphatic hydrocarbon of 600-100,000 average molecular weight and mineral lubricating oil which comprises reacting at a temperature in the range of 150-325° F. and in the presence of said diluent said reactants (a), (b), (c) and (d) in the respective molar ratio of 1.0:0.1-1.0:1.0-10:0.014-1.0 and then further reacting (e) 2-6 moles additional formaldehyde per mole of reactant (a) at a temperature in the range of 275-375° F. while blowing with inert stripping gas until the resultant product is dehydrated, wherein the amount of said diluent used provides 10-70 weight percent of said Mannich product as solute.

30 10. The method of claim 9 wherein the hydrocarbon diluent is butene polymer derived hydrocarbon of about 1500 number average molecular weight and SAE-5W oil, reactant (a) is about 1500 number average molecular weight polybutyl-substituted phenol, (b) is tetraethylene pentamine, (c) is formaldehyde, (d) is oleic acid and (e) is paraformaldehyde and wherein the amount of said diluent provides 40 weight percent of said Mannich product as solute.

#### References Cited

#### UNITED STATES PATENTS

|           |         |                       |            |
|-----------|---------|-----------------------|------------|
| 3,326,801 | 6/1967  | Schlobohm et al. ____ | 260-404.5  |
| 3,368,972 | 2/1968  | Otto _____            | 252-51.5 R |
| 3,442,808 | 5/1969  | Traise et al. _____   | 252-51.5 A |
| 3,216,936 | 11/1965 | Le Suer _____         | 260-404.5  |
| 2,276,309 | 3/1942  | Hummel et al. _____   | 260-404.5  |
| 3,280,970 | 10/1966 | Cizek _____           | 260-404.5  |
| 3,036,003 | 5/1962  | Verdol _____          | 252-51.5 R |
| 2,992,230 | 7/1962  | Lescisin _____        | 260-404.5  |
| 2,765,325 | 10/1956 | Niederhauser _____    | 260-404.5  |

GLENNON H. HOLLRAH, Primary Examiner

65 U.S. Cl. X.R.

252-51.5, 51.5 A; 260-247.7, 249.6, 293.89, 293.9, 309, 309.7, 326.5, 326.8, 404, 561 R, 561 N, 562 R, 562 P

UNITED STATES PATENT OFFICE  
CERTIFICATE OF CORRECTION

Patent No. 3,787,458 Dated January 22, 1974

Inventor(s) Edmund J. Piasek and Robert E. Karll

It is certified that error appears in the above-identified patent and that said Letters Patent are hereby corrected as shown below:

Column 5, Line 49 - bis Mannich should be bis-Mannich

Column 8, Line 4 - c.f.h. should be C.F.H.

Column 8, Line 47 - c.f.h. should be C.F.H.

Column 9, Line 27 - 0 should be 1.0

Signed and sealed this 29th day of October 1974.

(SEAL)  
Attest:

McCOY M. GIBSON JR.  
Attesting Officer

C. MARSHALL DANN  
Commissioner of Patents